

# UNITED STATES PATENT OFFICE.

ROBERT J. TILFORD AND HENRY M. REDEMAN, OF LOUISVILLE, KENTUCKY,  
ASSIGNORS TO THE REDEMAN - TILFORD STEEL COMPANY, OF SAME  
PLACE.

## MANUFACTURE OF STEEL.

SPECIFICATION forming part of Letters Patent No. 397,478, dated February 5, 1889.

Original application filed July 25, 1888, Serial No. 281,018. Divided and this application filed November 13, 1888. Serial No. 290,738. (No specimens.)

*To all whom it may concern:*

Be it known that we, ROBERT J. TILFORD and HENRY M. REDEMAN, citizens of the United States, residing at Louisville, Jefferson county, Kentucky, have invented new and useful Improvements in the Manufacture of Steel, of which the following is a specification.

Our invention relates to certain new and useful improvements in the treatment of crude or low-grade steel to produce a refined or high-grade steel.

The most successful method of producing low-grade steel is that known as the "Bessemer" process, described in his patent of 1855; but this product, as is well known, is suitable chiefly for railways, axles, and like uses, and is totally unsuited for structures, machinery, and tool purposes unless puddled, hammered, and rolled, for the reason that in its normal state it is too soft, and when hardened it becomes too hard and brittle for the purposes stated. It was the recognition of these inherent defects in the Bessemer and low and medium grade steel which led us to the investigation of the subject which has developed our present invention, the object of which is the production at slight cost and a minimum degree of labor of a higher grade and more refined steel by treating the Bessemer and other low and medium grades steel in such manner as to produce a molecular change from a coarse grain to a fine grain and silky fracture, to increase the tensile strength, elasticity, toughness, and ductility, and to greatly increase the carbon. We have found from experience that uniform results in all instances flow from the treatment of metals having like properties.

With these ends in view our invention consists in heating the metal to be treated to a white heat, and then submerging the same in a bath of glycerine and water having added thereto spirits of niter, aqua-ammonia, chloride of ammonium, sulphate of zinc, sulphate of alumina and ammonia, substantially as will hereinafter be more particularly set forth.

In some instances we employ simply glycerine and water for the treatment of the metal;

but we desire to say that we lay no claim 50 herein for such bodies alone, as they are covered by the first divisional application of our original application, Serial No. 281,018, filed July 25, 1888, which divisional application is filed of even date herewith, this application 55 constituting the second division of our original application referred to. Neither do we lay any claim to the broad or generic idea of heating low-grade steel to a degree of heat represented by white heat, and then subjecting the metal so heated to a liquid bath, (in contradistinction to the dry or cementation process,) in which hydrocarbon or other similar gases are generated by contact with the heated metal and bath, as this last-named 65 matter forms the subject of our said original application.

In the practice of this our present invention we employ the several chemical bodies in about the following proportions, to wit: 70 Spirits of niter, one and a half (1½) ounce; aqua-ammonia, one and a half (1½) ounce; chloride of ammonium two (2) ounces; sulphate of zinc, one and a half (1½) ounce; sulphate of alumina and ammonia, one and a 75 half (1½) ounce; glycerine, three (3) ounces; water, one-half (½) gallon.

We of course do not wish to confine ourselves to the exact proportions named, as they may be varied within reasonable limits and 80 yet produce the same general results; but we have found from long experience and repeated tests and experiments that the proportions given produce the best results. In preparing the bath we preferably first powder or granulate the chemicals and mix the same thoroughly and intimately with the glycerine until well dissolved, and we then add to the bodies so compounded the necessary quantity of water. It will also be understood that we 85 do not wish to confine ourselves to the exact degree of heat imparted to the metal, as that may be varied slightly, so long as the results desired are obtained.

We have of course been unable to analyze 95 the gases resulting from the contact of the hot-metal body with the bath, but are led to believe that they constitute a hydrocarbon

gas which has a strong affinity for the metal, and that the latter, being in a heated state, is in such a physical condition as to readily take up or absorb such gas; but as to the fact 5 that the metal is highly improved we have no doubt whatever, as has been demonstrated by all the well-known scientific and mechanical tests.

It will be understood, of course, that when 10 the treatment is applied adjacent to the furnaces where the low-grade steel is manufactured the ingots may be treated without re-heating, and thus the expense of such reheating is avoided. After the metal has been 15 subjected to the treatment in the bath described it is allowed to cool in the ordinary manner, and it may afterward be subjected to any ordinary hardening or tempering process, and the temper may, if necessary, be 20 drawn and again restored without at all affecting the other properties acquired from the bath.

We are of course aware that the quality 25 of Bessemer and other low and medium grade steel may be improved by what is known as the "dry" or "cementation" process, which requires a large expenditure of skilled labor and great length of time, and that, too, without 30 always securing uniform and satisfactory results.

We desire it to be distinctly understood 35 that we lay no claim to the broad idea of increasing the quality of steel by subsequent treatment, as that has been heretofore done, especially by what is known as the "cementation process," which may be termed a "dry process," our invention differing from such process in the particular that it requires a period of time amounting to a small percentage 40 of the time required in the cementation or dry process, and is in contradistinction to such process essentially a liquid or wet process, the former requiring many days, while the latter involves only a few minutes.

45 As before stated, we wish it to be understood that the chief feature of our process involves the employment of a bath having as its base glycerine and water, for in the use of these two bodies we accomplish desirable and important 50 proved results; but the addition to the glycerine and water of spirits of niter, aqua-ammonia, chloride of ammonium, sulphate of zinc, and sulphate of alumina and ammonia produce better and enhanced results; hence we

do not wish to confine ourselves to the use of a bath embodying all the bodies named.

Our invention or process is distinguished from processes for tempering steel in oil in that by our process the nature, the physical construction, and the molecular or granular 60 construction of the metal are completely changed, whereas the tempering of steel in oil, as practiced by some processes, simply tempers the metal more slowly than is done by tempering in water and other properties, 65 leaving the metal less hard but somewhat tougher than water-tempered material. The changes caused by the oil-tempering process are merely temporary, and do not change the physical or granular construction of the metal, 70 and such changes as are caused thereby can be readily neutralized by reheating and allowing the metal to cool. The changes caused by treatment by our process are permanent, and cannot be removed by any known treatment or process without entirely destroying 75 the steel properties of the metal by burning.

By our invention we greatly increase the tensile strength and elasticity, and yet do not 80 destroy the per cent. of reduction of ductility, while with ordinary tempering the tensile strength and elasticity are greatly increased, but the per cent. of reduction and ductility is very much impaired.

Having thus described our invention, what 85 we claim as new, and desire to secure by Letters Patent, is—

The process herein described for converting steel, which consists in first heating the metal to be treated to a white heat, and then 90 while so heated submerging the same in a liquid bath consisting of glycerine and water in the proportion of three ounces of the former and one-half gallon of the latter, combined with spirits of niter, one and a half ounce; 95 aqua-ammonia, one and a half ounce; chloride of ammonium, two ounces; sulphate of zinc, one and a half ounce; sulphate of alumina and ammonia, one and a half ounce, substantially as hereinbefore set forth.

In testimony whereof we have hereunto set 100 our hands in the presence of two subscribing witnesses.

ROBERT J. TILFORD.  
HENRY M. REDEMANN.

Witnesses:

H. J. TILFORD,  
DAVID BARTLEY.